

Oct. 11, 1932.

R. S. VON HAZMBURG

1,881,985

METHOD AND MEANS FOR MANUFACTURE OF PAPER

Filed April 6, 1931



Inventor:  
Romulus S. Von Hazmburg.

By John H. Miller  
Attorney.

## UNITED STATES PATENT OFFICE

ROMULUS S. VON HAZMBURG, OF CHESTER, PENNSYLVANIA, ASSIGNOR TO SCOTT  
PAPER COMPANY, A CORPORATION OF PENNSYLVANIA

## METHOD AND MEANS FOR MANUFACTURE OF PAPER

Application filed April 6, 1931. Serial No. 530,875.

My invention embodies method and means for eliminating the coagulating or grouping of impurities from the paper stock at or before the time it is delivered to the wire of the paper making machine, so that their actual presence is assured in such form as will prevent them operating to deface or clog the wire and thus cause the paper produced to be defective by reason of the resulting presence of holes at intervals apart formed through the body of the paper web.

All paper pulps contain more or less resinous material, some of which gives considerable trouble in paper making. This trouble is commonly due to the presence of pitch in the pulp. This resinous material or pitch is originally a constituent of wood and is associated in the fibers of the pulp. The resinous or pitch material is separated from the fibers by beating, jordaning, pressing or other mechanical process to which the fibers are subjected during paper stock making. The pitch separates out of the pulp as a milky suspension in the "white water" and may be of varying degrees of sub-division, and moreover behaves as a typical colloidal solution. During the processing of the fiber, the colloidal solution of pitch takes on a negative charge which prevents the minute particles of resinous material from adhering to the fiber. Due to the constant mixing, however, this colloidal solution of pitch coagulates into larger particles which can then be noticed as adhering lumps or splotches on the wire, felts and press rolls, of the Fourdrinier, causing them to operate defectively in the other wise normal operation of the paper making machines.

A typical colloidal solution of a finely suspended solid in a fluid bears an electrical "charge". Such solutions are stable until something neutralizes the "charge", causing a precipitation or flocculation of this suspended material in the solution. There are several ways by which this effect may be brought about; one is chemically performed by adding a colloidal solution having an opposite electrical charge, and another is by causing the solution to be brought into contact with grids or plates immersed therein,

said solution having a static potential, as preferred.

I have found by experiment that when "white water" is subjected to a static potential, the milky suspension is speedily flocculated, leaving a clear supernatent liquid; and that the desired result is secured by the employment of relatively high voltages in a shorter time; and while I do not limit myself to any particular voltages, I have found excellent results to be obtained with the use of 125 volts.

I have also determined that by the employment of terminal plates immersed in a circulating mass of a paper pulp, and said plates alternately positively and negatively charged with an electric current, the effect upon the pulp determined at the beginning and at the ending of the electric treatment of the pulp indicated that very little of the pitch separated from the fiber of the pulp; whereas in tests made upon the pulp without the employment of the electric charge, a materially larger amount of the pitch was beaten out or separated from the pulp and which by coagulation, increases into larger particles or masses which separate from the pulp and become deposited or lodged upon the wire, felts and other parts of the paper making machine, with the result that the paper product as made will contain more or less holes or defects in the web prior to passing to the driers.

The ability to eliminate the cause of these defects in the finished product and to prevent recurrence in an objectionable degree is far reaching because otherwise the defects due to the soiling of the wire by the pitch deposits will continually repeat themselves with each revolution of the wire apron and will gradually increase the number of defects per square yard of the paper web produced.

This defective operation is more especially due to the fact that when the particles, lumps or splotches of colloidal substances adhere to the surface of the wire apron of the Fourdrinier, said deposits, to the extent of their presence, cause the paper to be formed in the web with apertures or holes of various

55

60

65

70

75

80

85

90

95

100

shapes, these defects being more apparent with papers of more or less of the tissue grades such as toilet papers.

In practice, the paper stock is caused to 5 flow through or between the grids or plates of different polarities which induces negative polarity in the pulp to become neutralized. This fine suspension of pitch or its equivalent can then insure adherence to the 10 fiber and be gradually eliminated with the paper without producing therein holes or other physical defects.

I have found that the electrical treatment 15 may be performed in the head box of a paper making machine, or in the beater, as preferred; and that the use of higher voltages produces the desired neutralizing effect in a shorter time. By way of example, I have further found that a voltage of 125 volts 20 gives desirable results.

For the purpose of illustrating my invention, I have shown in the accompanying drawing the embodiment thereof which is at present preferred by me, since the same is 25 in form to give satisfactory and reliable results, but it is to be understood that the several instrumentalities of which my invention consists can be variously arranged and organized and that my invention is not limited 30 to the precise arrangement and organization of the instrumentalities herein shown and described.

By way of illustration and not as a limitation, I have shown in the drawing, a head 35 box A of a paper making machine provided with grids or plates B and C, respectively charged with opposite polarities through the mediation of any suitable source of electric current, preferably from a continuous current dynamo D and circuits E and F therefrom and respectively connected to and energizing the grids or plates. G represents the breast roll and H the wire of a Fourdrinier equipment of a paper making machine.

45 Instead of neutralizing the polarity of the pitch solution in the pulp in the head box, the neutralizing may be performed at any stage, as for example, in the beating engine, in the jordan, or the pressing operations, in 50 which the wood fibers are subjected to preliminary or preparatory treatment prior to the actual making of the paper. It is also to be understood that my invention includes the treatment of a mix furnished or formed of 55 sulphite and ground wood.

I have described my improved method and means in that particularity which I deem to be the best exposition of my invention, and that which I prefer in commercial practice, 60 but I do not restrict or confine myself to the minor or secondary details, as such are susceptible of modification, which may be resorted to as a matter of mechanical skill and without a departure from the spirit of the 65 invention.

I claim:

1. The herein described step in the manufacture of paper in web form which consists in forming a paper pulp and neutralizing the normal electric charge thereon by passing the 70 said paper pulp over electric charging means in communication with a source of electric energy and thereafter transforming the paper pulp into web form.

2. The herein described step in the manufacture of paper in web form which consists in subjecting the paper pulp containing resinous matters over electrically energized conducting surfaces for neutralizing the electric charge normally existing upon the pulp 80 and thereafter forming the neutralized pulp into paper in web form.

3. In paper making apparatus, the combination in a paper making machine including pulp supplying means, with means in the 85 path of the paper pulp supplied to the machine for neutralizing the static charge upon the pulp.

4. In a paper making apparatus, the combination with a Fourdrinier machine, of a 90 head box, and means for supplying an electric charge to the head box for neutralizing the electric charge upon the paper pulp being supplied to the wire apron.

5. The invention stated in claim 4, where- 95 in further, the neutralizing means comprises two grids respectively in contact with the paper pulp being supplied through said head box.

In testimony of which invention, I here- 100 unto set my hand.

ROMULUS S. von HAZMBURG.

101

102

103

104

105